

April 18, 1933.

A. G. ADAMSON

1,904,113

FILM FOR PHOTOGRAPHIC PURPOSES

Filed Sept. 11, 1931

*Core layer of gelatine rendered insoluble  
by formaldehyde or other agent  
(may contain glycerine)*



Inventor  
ANDREW GEORGE ADAMSON

By *Douglas Dowell*  
Attorneys

## UNITED STATES PATENT OFFICE

ANDREW GEORGE ADAMSON, OF LONDON, ENGLAND, ASSIGNOR TO W. M. STILL & SONS LIMITED, OF LONDON, ENGLAND, AND HIMSELF

## FILM FOR PHOTOGRAPHIC PURPOSES

Application filed September 11, 1931, Serial No. 582,411, and in Great Britain September 13, 1930.

The object of the present invention is to provide an improved photographic film of non-inflammable character adapted particularly for use in kinematographic apparatus.

5 A non-inflammable photographic film for use in kinematographic apparatus has long been sought, but so far, all such films as have satisfied requirements regarding non-inflammability have been defective in some other 10 respect, the most general defects being brittleness or lack of permanent flexibility and a tendency to react with the chemical constituents of the photographic image, which is thus spoiled.

15 A film embodying this invention, which is non-inflammable, flexible, transparent, substantially colorless and free of any danger of affecting the photographic image, is illustrated by the attached drawing, showing the 20 same in longitudinal section on a greatly enlarged scale.

Said film according to the invention consists in a thin core layer 1 of insoluble gelatine, coated on each side with a thin layer or 25 coating 2 of rubber, which in its turn is covered with an outer layer or coating 3 of celluloid, collodion or other varnish.

The purpose of the layers of rubber and 30 varnish is to provide a complete inseparable coating protecting the central or core film from any action by water or the various salts used in the development and fixing of the 35 photographic image, and adapted to receive on one side the sensitized emulsion without risk of the photographic image being detrimentally affected. The completed film, although it has a coating of a highly inflammable character such as celluloid, remains 40 non-inflammable, that is to say, when a flame is applied to the film or it is highly heated, all that happens is that the film curls up and hardens but does not ignite.

In carrying out the invention the following procedure may be adopted.

45 A warm solution of gelatine in water, to which a very small proportion of formaldehyde has been added (for instance about 1% of a 40% solution of formaldehyde) is flowed or poured on to a level travelling 50 metal band, on which it is carried in the form

of a film through a cooling chamber, where the gelatine sets and becomes insoluble and is then carried on into a current of warm air whereby it is dried. In some cases, to hasten the drying, the gelatine film may be drawn 55 through alcohol before being subjected to warm air. Instead of formaldehyde, other agents such as alum may be used to render the gelatine insoluble or practically non-absorbent.

To improve the pliability of the core layer, the solution may contain a trace of glycerine but it is found that the formaldehyde or alum not only renders the gelatine film insoluble but also toughens it and prevents its becoming 60 brittle. The temperature of the solution may be about 100° F.

In order to ensure regularity in the thickness of the core layer and to prevent flooding, the gelatine is extruded or delivered through 70 a suitable die onto the metal band at a temperature only a few degrees above its setting point and under such pressure as the speed of the moving metal band may require. The metal band, before it reaches the die, is 75 cooled considerably below the setting point of the gelatine, so that the surface of the gelatine in contact with the cool metal will set quickly and prevent flooding, while the main bulk of the gelatine will remain fluid enough 80 to find its own level, the band then carrying it on through the cooling chamber to finally set the whole.

The gelatine supporting surface of the metal band is next highly polished and 85 treated with a solution of wax in benzole or the like, so that after the gelatine film has been finally dried, it can be easily stripped off. The film of gelatine is then thinly coated on both sides with rubber varnish, 90 which may consist of a small percentage (say 3%) of pure rubber dissolved in fine petrol, and then on both sides coating with a varnish, which is preferably celluloid varnish. The rubber solution penetrates the 95 gelatine and the celluloid varnish adheres firmly to the rubber coated surface. After these varnishes have thoroughly dried, the film may be passed between highly polished pressure rollers to ensure a bright surface 100

and improve the adhesion of the separate layers.

It is preferred to use as the outer protecting medium a solution of celluloid such as 5 now used in making films, because although highly inflammable in itself, it imparts to the film, surfaces having the same other characteristics as an ordinary celluloid film. Collodion varnish may be used instead of celluloid varnish, as the outer coating.

Instead of adding the formaldehyde or other agent to the gelatine solution, the set gelatine film may be drawn through or immersed in an aqueous or alcoholic solution 15 of formaldehyde or other agent which also will render it insoluble without reducing its transparency or flexibility.

A coat of sensitized gelatine emulsion can be applied to a film according to this invention 20 in the ordinary way and the film can then be dealt with in the same way as a celluloid film without risk of the ultimate photographic image being affected, or of the coatings of rubber and celluloid separating from 25 each other or from the gelatine core, while the transparency, flexibility, colourlessness and durability of the film are adequate for all ordinary purposes.

What I claim is:—

30 1. A non-inflammable photographic film, which consists of a core layer of gelatine, rendered insoluble and coated on each side first with rubber and then with another protecting medium such as celluloid.

35 2. A non-inflammable photographic film comprising a core layer of gelatine, rendered insoluble by a substance, and having a coating of rubber varnish on each side with an outer coating of another protective medium 40 such as celluloid thereon.

45 3. A non-inflammable film for photographic purposes, which consists of a core layer of gelatine, rendered insoluble by a substance; the same being coated on each side with a thin sub-surface of rubber varnish and with a thin outer surface of another protecting medium such as celluloid.

50 4. A non-inflammable photographic film, which consists of a core layer of gelatine, rendered insoluble by formaldehyde and coated on each side first with rubber and then with another protecting medium such as celluloid.

55 5. The process of making a non-inflammable film for photographic purposes, which consists in first forming a core layer of gelatine from a warm aqueous solution containing a small proportion of an agent adapted to render the gelatine insoluble, cooling and drying the gelatine core layer, applying to each side of said layer a coating of rubber solution and thereafter applying thereto a coating of a celluloid solution.

60 6. The process of making a non-inflammable film for photographic purposes, which

consists in first forming a core layer of gelatine from a warm aqueous solution containing a small proportion of formaldehyde, cooling and drying the gelatine core layer, and coating both sides thereof first with a 70 rubber varnish and then with a celluloid varnish.

7. The process of making a non-inflammable film for photographic purposes, which consists in first forming a core layer of gelatine from a warm aqueous solution containing a small proportion of formaldehyde and a trace of glycerine, cooling and drying the gelatine core layer, coating both sides thereof with a rubber varnish, and then coating the 80 same with a celluloid varnish.

Signed at London, England, this 19th day of August, 1931.

ANDREW GEORGE ADAMSON.

85

90

95

100

105

110

115

120

125

130